

Oct. 9, 1973

M. F. LITTMANN

3,764,406

HOT-WORKING METHOD OF PRODUCING CUBE-ON-EDGE-ORIENTED  
SILICON-IRON FROM CAST SLABS

Filed Nov. 4, 1971

2 Sheets-Sheet 1



FIG. 1



FIG. 2

INVENTOR:

MARTIN F. LITTMANN

BY

*Melville, Strasser, Foster and Hoffman*  
ATTORNEYS

Oct. 9, 1973

M. F. LITTMANN  
HOT-WORKING METHOD OF PRODUCING CUBE-ON-EDGE ORIENTED  
SILICON-IRON FROM CAST SLABS

3,764,406

Filed Nov. 4, 1971

2 Sheets-Sheet 2



FIG. 4



FIG. 5



FIG. 3

INVENTOR:

MARTIN F. LITTMANN

BY *McEvill, Shasser, Foster and Hoffman*  
ATTORNEYS

1

3,764,406  
**HOT-WORKING METHOD OF PRODUCING CUBE-ON-EDGE ORIENTED SILICON-IRON FROM CAST SLABS**  
Martin F. Littmann, Middletown, Ohio, assignor to  
Armco Steel Corporation, Middletown, Ohio  
Filed Nov. 4, 1971, Ser. No. 195,553  
Int. Cl. H01f 1/04  
U.S. CL. 148—111 8 Claims

## ABSTRACT OF THE DISCLOSURE

A process for the production of cube-on-edge silicon-iron sheet stock having uniformly good magnetic properties, comprising melting, refining, casting into slabs, hot reducing to hot rolled thin band, removing the hot mill scale, cold reducing to final thickness in one or more stages, decarburizing and recrystallizing in a wet hydrogen anneal, coating with a separator and annealing in hydrogen above about 1100° C. The cast slabs are initially hot reduced at least 5% at a temperature of 750° to 1250° C., then heated above 1350° C. and hot rolled to a thickness of 2.5 mm. or less. The initial hot reduction produces a structure which prevents excessive grain growth during the subsequent heating and hot rolling steps.

## BACKGROUND OF THE INVENTION

### (1) Field of the invention

This invention relates to a method of producing oriented silicon-iron sheet or strip for magnetic purposes. The orientation with which the present invention is concerned is that wherein the grains or crystals are oriented in the cube-on-edge position, i.e. designated (110)[001] in accordance with the Miller Indices. More particularly, the invention relates to a method of producing grain-oriented silicon-iron sheet or strip containing from about 2% to 4% silicon of uniformly excellent magnetic properties. Although not so limited, the invention has particular utility in the production of grain-oriented silicon-iron sheet or strip wherein the molten steel is strand or continuously cast into a continuous slab of thickness suitable for direct hot rolling.

### (2) Description of the prior art

Cube-on-edge oriented silicon-iron sheet or strip is generally made by a series of steps including melting, refining, casting and hot reducing ingots or slabs to hot rolled bands of about 2.5 mm. thickness or less. After annealing and scale removal, the hot rolled band is cold reduced in one or more stages, with intermediate anneals if necessary, to a final thickness of about 0.25 to about 0.35 mm. The strip is then usually recrystallized and decarburized at final thickness by a continuous anneal in a wet hydrogen atmosphere. Finally, the strip is coated with an annealing separator and box annealed for several hours in dry hydrogen at a temperature above about 1100° C.

As is well known, two conditions must be satisfied prior to the high temperature portion of the final box anneal in order to obtain material having a high degree of cube-on-edge orientation, viz:

(1) A suitable structure of completely recrystallized grains with a sufficient number of these grains having the final cube-on-edge orientation;

(2) The presence of inhibitors in the form of small, uniformly distributed inclusions which restrain primary grain growth in the early portions of the anneal until a vigorous secondary growth occurs during the latter, high temperature portion of the anneal.

During the above mentioned secondary grain growth portion of the anneal, the cube-on-edge grains consume

2

other grains in the matrix having a different orientation.

The primary grain growth inhibitor, which must be present in the form of small, uniformly distributed inclusions, is usually manganese sulfide, but other inhibitors, e.g., manganese selenide, aluminium nitride, or mixtures thereof, may also be used for this purpose.

U.S. Pat. 2,599,340, issued June 3, 1952, to M. F. Littmann and J. E. Heck, discloses a process for the production of cube-on-edge silicon-iron wherein slabs rolled from ingots are heated to a temperature above about 1260° C., and particularly from about 1350° to about 1400° C. prior to hot rolling. This heating step not only prepares the metal for hot rolling but also dissolves the inhibitor present therein so that upon subsequent hot rolling the inhibitor is precipitated in the desired form of small, uniformly distributed inclusions, thereby satisfying one of the two essential conditions for obtaining highly oriented cube-on-edge material.

The practice of heating an ingot, or the product of an ingot rolled in to slab form, to a temperature above about 1260° C. and up to 1400° C. prior to hot rolling has been widely adopted and is currently in use.

Strand casting into a continuous slab or casting into individual slabs of a thickness suitable for direct hot rolling is now being used for making ferrous sheet stock. The term slab as used herein is intended to include cast bodies ranging in thickness from about 10 to about 30 cm. These casting techniques are advantageous in that they avoid the loss of material from the butt and top portions of conventional ingots, which ordinarily must be cropped. For example, slabs of silicon-iron are strand cast into a thickness of 15 cm., cut to suitable length and reheated to about 1350° to 1400° C. in order to dissolve the inhibitor prior to hot rolling. However, the degree of the cube-on-edge orientation of the product of strand cast slabs has tended to be much more variable than material produced from ingots, especially across the width of the strip.

Lack of uniformity and frequent inferiority in magnetic properties of material produced by strand casting have hitherto limited the utility of strand casting despite the advantages over conventional production from ingots.

## SUMMARY

It has been ascertained that a principal cause of the above mentioned variable and often inferior development of cube-on-edge texture results from excessive grain size in the slab, which occurs as a result of reheating above about 1300° C. prior to hot rolling. Strand cast slabs in the as cast condition have a crystal structure which upon reheating above 1300° C. exhibits grain growth to an average diameter of about 25 mm. (about 0.5 to 1.0 ASTM grain size at 1X). By way of comparison, the average grain diameter in slabs rolled from ingots, after reheating to about 1300° C., is about 10 mm.

According to the present invention, it has been found that limiting the grain size in the slabs, after reheating to high temperature and prior to hot rolling, to a diameter not exceeding that represented by about 4.5 ASTM at 1X (corresponding to an average diameter of about 7 mm. or less) has a beneficial effect on the development of cube-on-edge texture in the final product. Apparently the smaller grain size promotes more complete recrystallization during the processing anneals subsequent to hot rolling.

It has now been discovered that control of the grain size in the slabs after the high temperature reheating can be achieved by hot reducing (prerolling) the cast slab by at least about 5%, before reheating, at a temperature below that at which excessive grain growth occurs. Ordinarily, excessive grain growth in the slab may begin between about 1260° and 1350° C. Hence, this initial hot

reduction is carried out within the range of about 750° to 1250° C., and preferably between about 850° and 1150° C.

The initial hot rolling step of the present invention results in a marked reduction in the size of the grains in the slab after reheating to about 1400° C. A hot reduction of about 25% results in a grain size after reheating of about 5 mm. average diameter (i.e. about 5-6 ASTM grain size at 1×). At least about 5% initial hot reduction is required. Reductions between about 10% and about 50% are preferred.

To the best of applicant's knowledge it has never previously been recognized that initial hot reduction of a silicon-iron cast slab would result in improved magnetic properties by control of grain size upon reheating to very high temperatures.

From the foregoing discussion it will be apparent that it is a primary object of the present invention to provide a process for the production of cube-on-edge oriented silicon-iron sheet stock of uniformly excellent magnetic properties from cast slabs.

#### BRIEF DESCRIPTION OF THE DRAWINGS

Reference is made to the accompanying drawings wherein:

FIG. 1 is a photograph at 0.5× magnification of a transverse section of a 15 cm. thickness strand cast slab in the as cast condition;

FIG. 2 is a photograph at 0.5× magnification of a transverse section of the strand cast slab of FIG. 1 after reheating to about 1400° C.;

FIG. 3 is a photograph at 0.5× magnification of a transverse section of a 20 cm. thickness strand cast slab of the same heat as FIG. 1 in the as-cast condition;

FIG. 4 is a photograph at 0.5× magnification of a longitudinal section of the slab of FIG. 3 after being hot reduced 25% in thickness at 1035° C., in accordance with the invention; and

FIG. 5 is a photograph at 0.5× magnification of a transverse section of the initially hot rolled slab of FIG. 4 after reheating to about 1400° C.

#### DESCRIPTION OF THE PREFERRED EMBODIMENTS

While the present invention is not so limited, its preferred embodiments will be described with reference to material strand cast into continuous slabs.

In an exemplary routing a charge is melted in conventional manner in an open hearth, electric arc furnace, or basic oxygen furnace, and tapped into a ladle to which

|                             |       | Percent |
|-----------------------------|-------|---------|
| Carbon                      | 0.034 |         |
| Manganese                   | 0.062 |         |
| Sulfur                      | 0.024 |         |
| Silicon                     | 3.17  |         |
| Balance substantially iron. |       |         |

For purposes of comparison, part of the heat of Example 1 was subjected to subsequent processing in accordance with the present invention and part in accordance with conventional practice. That portion processed in accordance with the present invention was strand cast to 20 cm. thickness, while that portion processed in accordance with conventional practice was strand cast to 15 cm. thickness. The two processes are summarized below in tabular form and designated as A and B respectively.

|    | A                                                                                      | B                                                                                      |
|----|----------------------------------------------------------------------------------------|----------------------------------------------------------------------------------------|
|    | Process of present invention                                                           | Conventional process                                                                   |
| 20 | 1... Shear slabs into appropriate lengths.                                             | 1... Shear slabs into appropriate lengths.                                             |
|    | 2... Heat slabs to 1,035° C.                                                           | 2... Reheat to 1,400° C.                                                               |
|    | 3... Hot reduce 25% to 15 cm. thickness.                                               | 3... Hot roll to 1.9 mm. thickness.                                                    |
|    | 4... Reheat to 1,400° C.                                                               | 4... Strip anneal at 975° C.                                                           |
| 25 | 5... Hot roll to 1.9 mm. thickness.                                                    | 5... Cold reduce to .264 mm. thickness (2 stages with intermediate anneal at 925° C.). |
|    | 6... Strip anneal at 975° C.                                                           | 6... Decarburize—strip anneal at 825° C. in wet hydrogen.                              |
|    | 7... Cold reduce to .264 mm. thickness (2 stages with intermediate anneal at 925° C.). | 7... Box anneal at 1,200° C. for 24 hours in dry hydrogen.                             |
| 30 | 8... Decarburize—strip anneal at 825° C. in wet hydrogen.                              |                                                                                        |
|    | 9... Box anneal at 1,200° C. for 24 hours in dry hydrogen.                             |                                                                                        |

#### Example 2

A heat was melted, refined and cast, in the same manner as that of Example 1, having the following composition:

|                             | Percent |
|-----------------------------|---------|
| Carbon                      | 0.030   |
| Manganese                   | 0.057   |
| Sulfur                      | 0.024   |
| Silicon                     | 3.15    |
| Balance substantially iron. |         |

Again, part of the heat was strand cast to 20 cm. thickness and processed further in accordance with the present invention (process A), while another portion was strand cast to 15 cm. thickness and processed further in accordance with conventional practice (process B).

The magnetic properties of the final products of the heats of Examples 1 and 2 produced by both processes A and B are compared in Table I.

TABLE I

| Example                | No. tests | Process A                 |         |           | Process B    |         |           |
|------------------------|-----------|---------------------------|---------|-----------|--------------|---------|-----------|
|                        |           | Permeability <sup>1</sup> |         | No. tests | Permeability |         | No. tests |
|                        |           | Range                     | Average |           | Range        | Average |           |
| 1-----                 | 20        | 1,820-1,840               | 1,833   | 22        | 1,745-1,840  | 1,808   |           |
| 2-----                 | 14        | 1,820-1,840               | 1,832   | 14        | 1,770-1,820  | 1,799   |           |
| Core loss <sup>2</sup> |           |                           |         |           |              |         |           |
| 1-----                 | 20        | .700-.755                 | .725    | 22        | .680-.885    | .757    |           |
| 2-----                 | 14        | .690-.750                 | .722    | 14        | .700-.855    | .777    |           |

<sup>1</sup> Permeability is indicated at H=10 oersteds.

<sup>2</sup> Core loss is indicated in watts per pound at 17 kilogausses and a frequency of 60 cycles per second.

all, or a substantial part of, the required silicon is added. The melt may then be refined, by procedures which may include vacuum degassing if desired. The melt is next transferred to a casting station and cast to a desired thickness, e.g. 15 or 20 cm.

#### Example 1

A heat was processed in the above described manner and strand cast into slabs having the following composition:

It will be apparent from Table I that material produced in accordance with the present invention exhibits a significant improvement both in average permeability and core loss, and more particularly in uniformity of these properties. The permeability of material produced by process A ranges between 1820 and 1840 with an average above 1830, as compared to permeability ranges of from 1745 to 1840 and an average of about 1804 for material produced from strand cast slabs in accordance with process B.

## Example 3

A heat was melted, refined and cast, in the same manner as that of Example 1, except that all the slabs were strand cast to 20 cm. thickness. The composition of the heat of Example 3 was as follows:

|                             | Percent |
|-----------------------------|---------|
| Carbon                      | 0.031   |
| Manganese                   | 0.055   |
| Sulfur                      | 0.024   |
| Silicon                     | 3.16    |
| Balance substantially iron. |         |

For purposes of comparison, part of the heat was subjected to subsequent processing in accordance with the invention and part in accordance with conventional practice. The two processes are summarized below and designated as C and D respectively.

| C                                                                                      |  | D                                                                                      |  |
|----------------------------------------------------------------------------------------|--|----------------------------------------------------------------------------------------|--|
| Process of present invention                                                           |  | Conventional process                                                                   |  |
| 1... Shear slabs into appropriate lengths.                                             |  | 1... Shear slabs into appropriate lengths.                                             |  |
| 2... Heat slabs to 1,035° C.                                                           |  | 2... Reheat to 1,400° C.                                                               |  |
| 3... Hot reduce 25% to 15 cm. thickness.                                               |  | 3... Hot roll to 1.9 mm. thickness.                                                    |  |
| 4... Reheat to 1,400° C.                                                               |  | 4... Strip anneal at 975° C.                                                           |  |
| 5... Hot roll to 1.9 mm. thickness.                                                    |  | 5... Cold reduce to .264 mm. thickness (2 stages with intermediate anneal at 925° C.). |  |
| 6... Strip anneal at 975° C.                                                           |  | 6... Decarburize—strip anneal at 825° C. in wet hydrogen.                              |  |
| 7... Cold reduce to .264 mm. thickness (2 stages with intermediate anneal at 925° C.). |  | 7... Box anneal at 1,200° C. for 24 hours in dry hydrogen.                             |  |
| 8... Decarburize—strip anneal at 825° C. in wet hydrogen.                              |  |                                                                                        |  |
| 9... Box anneal at 1,200° C. for 24 hours in dry hydrogen.                             |  |                                                                                        |  |

## Example 4

A heat was melted, refined, cast and subsequently processed in the same manner as Example 3, having the following composition:

|                             | Percent |
|-----------------------------|---------|
| Carbon                      | 0.031   |
| Manganese                   | 0.055   |
| Sulfur                      | 0.026   |
| Silicon                     | 3.15    |
| Balance substantially iron. |         |

Again, all slabs were cast to 20 cm. thickness, with part of the heat processed in accordance with the present invention, and another portion processed in accordance with conventional practice.

The magnetic properties of the final products of the heats of Examples 3 and 4 produced by both processes C and D are compared in Table II.

TABLE II

| Example                | Process C |                           |         | Process D |              |         |
|------------------------|-----------|---------------------------|---------|-----------|--------------|---------|
|                        | No. tests | Permeability <sup>1</sup> |         | No. Tests | Permeability |         |
|                        |           | Range                     | Average |           | Range        | Average |
| 3-----                 | 24        | 1,820-1,850               | 1,835   | 24        | 1,760-1,840  | 1,799   |
| 4-----                 | 16        | 1,810-1,830               | 1,830   | 24        | 1,785-1,840  | 1,818   |
| Core loss <sup>2</sup> |           |                           |         |           |              |         |
| 3-----                 | 24        | .685-.740                 | .707    | 24        | .705-.870    | .777    |
| 4-----                 | 16        | .665-.735                 | .712    | 24        | .675-.805    | .736    |

<sup>1</sup> Same as Table I.

<sup>2</sup> Same as Table I.

Since all slabs had the same initial thickness in processes C and D, it will be apparent that the hot rolling after reheating (step 3 in process D) involved a greater reduction in thickness in the conventional process than the corresponding step 5 in process C in view of the fact that the slab has already been hot reduced to 15 cm. thickness in step 3 of process C.

The data of Tables I and II show that the magnetic properties obtained from slabs reheated to very high temperature are similar for slabs cast to 15 cm. and 20 cm. thickness and processed in the conventional manner. It is believed that initial slab thickness, at least within the

range of about 10 cm. to about 30 cm. thickness, has little or no effect on the response to the initial low temperature hot reduction, so long as this initial reduction in thickness is at least about 5%.

From Table II it is apparent that relatively poor and non-uniform results are obtained by the conventional process for slabs cast to 20 cm. thickness, whereas uniform and superior properties are obtained by the process of the present invention.

A substantial number of coils has been processed to a final gauge of .264 mm. in accordance with the present invention, including the examples shown above, and 98.4% of the test values of permeability at H=10 were 1820 or higher and 62.8% of the values were 1840 or higher.

FIGS. 1-5 are photographs of etched sections of strand cast slabs of Example 2 produced both by process A and process B.

Referring to FIG. 1, which is a transverse section at 0.5 $\times$  magnification of a slab cast to 15 cm. thickness, it will be noted that a columnar grain structure extends from each surface inwardly almost to the center of the slab, with a relatively narrow core or band of equiaxed grains at the center. FIG. 2 illustrates the effect of reheating the slab of FIG. 1 to 1400° C., in accordance with conventional practice. It will be noted that excessive growth both of the columnar and equiaxed grains has occurred, the average grain size being about 0.5 to 1.0 ASTM at 1 $\times$  magnification (corresponding to an average grain diameter of about 25 mm.).

FIG. 3 is a transverse section at 0.5 $\times$  magnification of a slab (of Example 2) cast to 20 cm. thickness. It will be noted that the structure is substantially identical to that of FIG. 1.

FIG. 4, which is a longitudinal section at 0.5 $\times$  magnification, illustrates the effect of initially hot reducing the slab of FIG. 3 by 25% at a temperature of 1035° C., in accordance with the present invention. It will be noted that the columnar grain structure is still evident after hot rolling and is somewhat distorted. However, a significant feature of the hot rolled slab at this stage is the appearance of numerous recrystallized grains, which are randomly dispersed throughout the interior of the slab. The appearance of the recrystallized grains at this stage depends upon the temperature of hot rolling and is not considered to be critical.

FIG. 5 is a transverse section at 0.5 $\times$  magnification of the initially hot rolled slab of FIG. 4 after reheating to 1400° C. It will be noted that reheating has resulted in the formation of a much smaller, equiaxed grain struc-

ture, of about 5-6 ASTM grain size at 1 $\times$ , i.e., an average grain diameter of about 5 mm. This is in marked contrast to the grain structure of FIG. 2, and is very significant in view of the fact that the slab of FIG. 2 and that of FIG. 5 were each subjected to the same reheat temperature of 1400° C.

It is believed that complete recrystallization takes place in the early stages of high temperature reheating from nuclei formed during the initial hot rolling of the cast slab. This recrystallization structure exhibits less grain growth during the completion of the slab reheating to 1400° C. than the original cast structure as shown in FIG. 2.

It is thus apparent that application of an amount of low temperature hot working sufficient to cause a marked reduction in the size of the grains of the slab after reheating to a temperature above about 1300° C. achieves the principal object of the present invention.

As indicated previously, the preferred range of initial hot reduction is from 10% to 50%. A 25% initial reduction was found to develop optimum grain refinement in the reheated slab. Reductions below 5% do not introduce sufficient energy to be beneficial. As percent reduction increases over 25%, the benefit as measured by grain size of the reheated slab gradually diminishes to the extent that about 50% reduction may be considered the practical upper limit of this invention. The preferred temperature range for the initial hot reduction is from 850° to 1150° C., as contrasted with the usual soaking pit temperature of 1230° C. for ingots which are rolled into slabs, which constitutes a reduction in excess of 70%.

Continuous casting installations are in operation which incorporate in-line hot reduction capability. In such an arrangement the residual heat of the cast slab may be sufficient to permit initial hot reductions within the ranges of the present invention. This could minimize or eliminate reheating of slabs for initial hot rolling.

Although in-line hot rolling is presently being used for strand cast plain carbon steel, this results in direct recrystallization of the grain structure, unlike the situation with silicon-iron wherein the original columnar grain structure is not broken up as a direct result of hot rolling but recrystallizes during reheating to very high temperature.

The benefits of the present invention are not dependent on composition, and may be realized with any inhibitor, e.g., manganese sulfide, manganese selenide, aluminum nitride, or mixtures thereof. By way of example, the skilled worker will recognize that heats may be processed to obtain uniform magnetic properties by selecting appropriate combinations of elements within the following ranges:

|           |                  |
|-----------|------------------|
| Carbon    | 0.02-0.05%.      |
| Manganese | 0.04-0.12%.      |
| Sulfur    | 0.015-0.035%.    |
| Silicon   | 2-4%.            |
| Nitrogen  | Less than 0.01%. |
| Aluminum  | Less than 0.04%. |

and balance substantially iron, all percentages being by weight.

As illustration, reference is made to U.S. Pats. No. 3,287,183 issued to Taguchi et al., and No. 2,867,557 issued to Crede et al., wherein two types of compositions are disclosed.

The embodiments of the invention in which an exclusive property or privilege is claimed are defined as follows:

1. A process for the production of cube-on-edge texture silicon-iron sheet stock containing from about 2% to about 4% silicon, comprising the steps of melting a charge of silicon-iron, casting the charge to produce a slab having a thickness of about 10 to about 30 centi-

meters, heating the slab to a temperature of at least about 750° C. but below about 1250° C., initially hot reducing the slab with a reduction in thickness of 5% to 50%, reheating the slab to a temperature between about 1260° and 1400° C. to obtain a grain diameter not exceeding that represented by about 4.5 ASTM at 1×, hot rolling the slab to a hot band, cold reducing to final gauge in at least one stage, decarburizing, and finally annealing under conditions which effect secondary recrystallization by causing cube-on-edge grains to consume other grains having a different orientation.

2. The process of claim 1, wherein said initial hot reducing step comprises a reduction in thickness of about 10% to about 50%.

3. The process of claim 2, wherein said hot reducing comprises a reduction in thickness of about 25%.

4. The process of claim 1, wherein said slab is heated to a temperature of from about 850° to about 1150° C.

5. The process of claim 1, including the step of strip annealing the silicon-iron after hot rolling to a hot band and before cold reducing to final gauge.

6. The process of claim 1, wherein said cold reducing step comprises cold rolling in at least two stages with an intermediate strip anneal between each stage.

7. Cube-on-edge texture silicon-iron sheet stock produced by the process of claim 1.

8. A process for the production of cube-on-edge texture silicon-iron sheet stock containing from about 2% to about 4% silicon, comprising the steps of melting a charge of silicon-iron, continuously casting the charge to produce a slab having a thickness of about 10 to about 30 centimeters, initially hot reducing the slab with a reduction in thickness of 5% to 50% while said slab retains the residual heat of the casting step at a temperature of at least about 750° C. but below about 1250° C., reheating the slab to a temperature between about 1260° and 1400° C. to obtain a grain diameter not exceeding that represented by 4.5 ASTM at 1×, hot rolling the slab to a hot band, cold reducing to final gauge in at least one stage, decarburizing, and finally annealing under conditions which effect secondary recrystallization by causing cube-on-edge grains to consume other grains having a different orientation.

#### References Cited

| UNITED STATES PATENTS |         |               |         |
|-----------------------|---------|---------------|---------|
| 3,144,363             | 8/1964  | Aspden et al. | 148-111 |
| 3,147,158             | 9/1964  | Fiedler       | 148-111 |
| 3,214,303             | 10/1965 | Fiedler       | 148-111 |
| 50 3,105,782          | 10/1963 | Walter        | 148-111 |
| 2,599,340             | 6/1952  | Littmann      | 148-111 |
| 2,473,156             | 6/1949  | Littmann      | 148-111 |

L. DEWAYNE RUTLEDGE, Primary Examiner

55 W. R. SATTERFIELD, Assistant Examiner

U.S. CL. X.R.

148-31.55, 110, 112